

W. A. INGHAM,  
PROCESS OF ROASTING ORES,  
APPLICATION FILED FEB. 21, 1918.

1,283,782.

Patented Nov. 5, 1918.



Inventor:  
William A. Ingham,  
by Hazard E. Miller  
Atty's.

# UNITED STATES PATENT OFFICE.

WILLIAM A. INGHAM, OF LOS ANGELES, CALIFORNIA.

## PROCESS OF ROASTING ORES.

1,283,782.

Specification of Letters Patent.

Patented Nov. 5, 1918.

Application filed February 21, 1918. Serial No. 218,462.

To all whom it may concern:

Be it known that I, WILLIAM A. INGHAM, a citizen of the United States, residing at Los Angeles, in the county of Los Angeles and State of California, have invented new and useful Improvements in Processes of Roasting Ores, of which the following is a specification.

My invention relates to a process of reducing ores.

It is an object of this invention to treat ores, especially sulfid ores so as to volatilize the metal sulfids in a roasting chamber under the exclusion of air and after egress from the roasting chamber, causing air to come in contact with the volatilized metal sulfid to convert the same to the metal oxid and sulfur dioxid and to provide a simple apparatus for carrying out this process.

My invention consists in the steps of the process as hereinafter described and claimed.

In the accompanying drawings which form a part of this specification, I have illustrated an apparatus used in connection with my process, and in which:

Figure 1 is a horizontal section on lines 1—1 of Fig. 2.

Fig. 2 is a vertical section on line 2—2 of Fig. 1.

Fig. 3 is a vertical section on line 3—3 of Fig. 1.

Fig. 4 is a vertical section on line 4—4 of Fig. 1, showing the bearings of the rotating table.

In the drawings, 10 indicates an annular furnace chamber surrounding a vertical stack or chimney 11 to which the same is connected by means of two oppositely arranged ports 12 and 13. 14 and 15 are vertical baffle walls extending from opposite sides of the stack 11. 16 and 17 indicate burner nozzles arranged at opposite sides and on the outer periphery of the furnace chamber 10. 19 is a rotary roasting table annular

in shape and strengthened by reinforcing radial ribs 19' on its under side. The table 19 is provided with rollers 20 adapted to travel on a grooved track 21 suitably secured to the stack 11. The outer end of the table

is provided on its under side with a rack 22 adapted to engage a series of pinions 23 mounted in suitable bearings 24 supported on the outer walls of the furnace chamber 10. 25 is a circular asbestos board adjacent

to the outer end of the rotating table 19 and on the under side thereof, and adapted

to keep fuel and waste gases from passing from the furnace chamber 10 past the rack 22 into the roasting chamber 26. 27 is a metal plate extending upwardly from the outer wall of the furnace chamber and forming the outer wall of the roasting chamber 26. 28 is an angle iron suitably fastened to the wall 27 and forming a horizontal flange 29 projecting inwardly and above the outer edge of the roasting table 19. This flange 29 serves to maintain the roasting table 19 in alinement with the pinions 24. The inner end of the roasting chamber 26 is formed by the stack 11 and the top 30 is built of any suitable refractory material.

On opposite sides of the stack 11 and extending therefrom to the outer periphery of the roasting chamber 26 are a pair of ore feeding devices 31 consisting of a hopper 32, a rotary water cooled cylinder 33 mounted on a shaft 33' and disposed in a water cooled casing 34. The rotary cylinder 33 forms with the wall of the hopper 32, adjacent thereto, a narrow feed slot 35. The ends of shaft 33' are mounted in movable bearings 50 whereby the cylinder 33 may be moved in relation to the hopper 32 to adjust the width of the feed slot 35. Power is transmitted by means of a pulley 36 connected with any suitable source of power, and secured to a drive shaft 37 suitably mounted. 38 is a gear wheel fast to shaft 37 and in mesh with idler gear 39 which in turn meshes with gear 40 mounted on shaft 41 secured to feed roller 33. On the inner end of shaft 37 a gear 42 is mounted which is in mesh with a drive gear 43 engaging the rack 22 fast on the roasting table 19.

The roasting table 19 rotates in the direction of the arrows shown in Fig. 1, and the ore distributed thereon is after the volatilization of the metal sulfids has taken place, removed by a series of parallel cleaning rods 44, whose ends are loosely mounted for vertical movement in slots 51 formed with vertical plates 52. The vertical plates 52 in which the inner ends of the cleaning rods 44 are mounted, are supported by a vertical partition wall 53 of refractory material, extending from the top 30 of the roasting chamber 26 and from the chimney 11 to the outer periphery of the roasting chamber. The lower ends of the walls 53 extend within a fraction of an inch of the roasting table 19, allowing just sufficient clearance for the layer of ore deposited on

said table to pass therebeneath, and preventing any escape of the vapors or entrance of air into the roasting chamber. It will be noted that the two partition walls 53 divide 5 the roasting chamber 26 into two chambers 261 and 262 so that my roasting chamber 26 is really composed of two chambers, each provided with its own ore feeding and ore removing devices. The rods 44 occupy the 10 space between the walls 53 and the ore feeding devices 31 adjacent thereto, and serve to scrape the treated ore from the roasting table 19 into an ore residue chamber 45.

The ore to be treated is ground to about 15 fifty mesh and deposited in a thin sheet by means of the ore feeding device 31 on to the roasting table 19. The degree of thickness of the layer of ore deposited on the roasting table 19 may be controlled by either increasing 20 or decreasing the speed of rotation of the roasting table 19 or increasing or decreasing the amount of ore through the ore feeding device 31 by adjusting the width of the ore feeding slot 35. The roasting table 19 is 25 heated to a temperature sufficient to volatilize the metal sulfid during its travel from the ore feeding device to the first set of ore residue cleaning rods 44 that it encounters. I have found that in cases where the thickness 30 of the layer of ore is 1/192 of an inch and the length of the layer 72 inches, the metal sulfids are completely volatilized in a roasting period of six seconds before they encounter the cleaning rods 44 that remove 35 the residue of the ore from the table 19 on to the scoria chambers 45. The metal sulfid vapors due to their own expansion, pass through outlet passages 46 arranged immediately above the burners 17 and are brought 40 in contact with air entering through a conduit 47 which will convert the metal sulfid into the metal oxid and sulfur dioxid, which are separated from each other by the usual methods.

45 It should be noted that with the exception of a small quantity of air which enters the roasting chamber 26 with the ground ore through the ore feeding device 31, the roasting of the ore takes place under the exclusion 50 of air within the roasting chamber 26. By reason of the fact that the layer of ore on the roasting table is exceedingly thin, which is preferably to a degree in which the ore particles are separate from each other, the metal sulfids are completely volatilized and the 55 rabbling of the ore required in the usual roasting process is dispensed with in my apparatus, as no sintering or fritting of the ore takes place, no oxids being formed within 60 the roasting chamber, except a negligible quantity due to the air admitted with the

ground ore. By my process, the volatile metallic contents of the ore are completely extracted.

In the old processes, in which ore is roasted 65 in the presence of air, it is necessary to rabble the ore to expose all the particles of the ore to the air for oxidation. This rabbling is entirely dispensed with in my process, since it depends upon the volatilization of 70 the metal, thus avoiding the rabbling and the loss of the ore that is carried away in the form of dust. Furthermore the volatilized metal subsequently recovered in the state of 75 an oxid is in a substantially pure state uncontaminated with ore dust.

I have intended my process principally for the roasting of ores containing sulfids of arsenic and antimony. It is obvious however, that the same may be applied to ores 80 containing metallic compounds which may be volatilized under the condition existing in the ordinary roasting furnace. My process is especially valuable in connection with gold and silver ores containing sulfids of 85 arsenic or antimony. As well known, gold ores which are to be treated by the cyanid process are penalized if such ores contain sulfid of arsenic or antimony. By subjecting such ores to preliminary roasting treatment 90 in accordance with my process, the objectionable antimony and arsenic compounds may be easily removed.

My process is a simple one and needs little 95 supervision or technical skill in operation. The apparatus is simple, and worn out parts may be easily replaced. Furthermore the contamination of the ore and ore products by the furnace gases is avoided.

Various changes in the steps of the process 100 and in the construction of the roasting furnace may be made without departing from the spirit of my invention, as claimed.

I claim:

1. A process of treating ores containing 105 antimony sulfids, comprising heating a thin layer of the ground ore in a closed roasting chamber to a temperature sufficient to volatilize the antimony sulfids, conducting the antimony sulfid vapors from the roasting 110 chamber, and oxidizing said vapors to form antimony oxid.

2. A process of treating ores containing metal sulfids, comprising heating a thin layer of the ground ore in a closed roasting 115 chamber to a temperature sufficient to volatilize the metal sulfid, conducting the metal sulfid vapors from the roasting chamber and oxidizing said vapors to form the metal oxid.

In testimony whereof I have signed my 120 name to this specification.

WILLIAM A. INGHAM.